

# UNITED STATES PATENT OFFICE.

AUGUST BUNGER, OF HOBOKEN, NEW JERSEY.

## BRONZING LIQUID.

1,220,947.

Specification of Letters Patent.

Patented Mar. 27, 1917.

No Drawing.

Application filed May 18, 1916. Serial No. 98,418.

*To all whom it may concern:*

Be it known that I, AUGUST BUNGER, a citizen of the United States, residing at Hoboken, in the county of Hudson and State of New Jersey, have invented certain new and useful Improvements in Bronzing Liquids; and I do hereby declare the following to be a full, clear, and exact description of the invention, such as will enable others skilled in the art to which it appertains to make and use the same.

The invention relates to a bronzing liquid for printers' ink.

The object of the present invention is the production of a bronzing liquid for use in connection with printing bronze powders and designed to be mixed with the bronze powders by pressmen when ready to put the mixture on a printing press.

The bronzing liquid consists of a mixture of rosin, a compound of lead, preferably lead oxid, manganese borate, olive or cotton seed oil, boiled linseed oil, printers' varnish and coloring matter consisting of printers' ink. The printers' ink is employed for imparting the desired tint or shade to the bronzing liquid for adapting the same for use in connection with the bronze powder with which it is to be mixed.

In preparing the composition I prefer the ingredients in about the following proportions; one part rosin, one part lead oxid, one part manganese borate, two parts olive or cotton seed oil, five parts boiled linseed

oil, five parts printers' varnish and five parts printers' ink.

The ingredients of the composition are thoroughly mixed and in the use of the bronzing liquid the latter is mixed with bronze powder to form a printing ink of the desired consistency for use on a printing press or analogous purpose.

What is claimed is:—

1. A bronzing liquid for admixture with bronze powder, said bronzing liquid including rosin, a compound of lead, a compound of manganese, a vegetable oil, printers' varnish and coloring matter.

2. A bronzing liquid for admixture with bronze powder, said bronzing liquid including rosin, a compound of lead, manganese, a vegetable oil, printers' varnish and printers' ink for producing the proper tint or shade.

3. A bronzing liquid for admixture with bronze powder, said bronzing liquid consisting of one part rosin, one part lead oxid, one part manganese borate, two parts cotton seed oil, five parts boiled linseed oil, five parts printers' varnish, and five parts printers' ink.

In testimony whereof I affix my signature in presence of two witnesses.

AUGUST BUNGER.

Witnesses:

JOHN VORRATH,  
FREDERICK HEIGIS.

Copies of this patent may be obtained for five cents each, by addressing the "Commissioner of Patents, Washington, D. C."